



US008067140B2

(12) **United States Patent**  
**Sensui**

(10) Patent No.: US 8,067,140 B2  
(45) Date of Patent: Nov. 29, 2011

- (54) **TONER FOR DEVELOPING ELECTROSTATIC IMAGE AND METHOD OF PRODUCING THE SAME**

(75) Inventor: **Keita Sensui**, Tokyo (JP)

(73) Assignee: **Zeon Corporation**, Tokyo (JP)

( \*) Notice: Subject to any disclaimer, the term of this patent is extended or adjusted under 35 U.S.C. 154(b) by 967 days.

(21) Appl. No.: 12/022,501

(22) Filed: Jan. 30, 2008

(65) **Prior Publication Data**

US 2008/0182189 A1 Jul. 31, 2008

(30) **Foreign Application Priority Data**

Jan. 31, 2007 (JP) ..... 2007-022493

(51) Int. Cl.

**G03G 9/08** (2006.01)  
(52) U.S. Cl. 430/108.2; 430/108.22; 430/137.15

**Field of Classification Search** 430/

#### (56) References Cited

U.S. PATENT DOCUMENTS

6.887.637 B2 \* 5/2005 Niwa ..... 430/108.22

## FOREIGN PATENT DOCUMENTS

JP 11-15192 A 1/1999  
JP 2000-3076 A 1/2000  
JP 2000-321809 A 11/2000

|    |             |    |        |
|----|-------------|----|--------|
| JP | 2001-117272 | A  | 4/2001 |
| JP | 2006-184687 | A  | 7/2006 |
| WO | 2005-081639 | A3 | 9/2005 |
| WO | 2005-091080 | A1 | 9/2005 |
| WO | 2007-010828 | A1 | 1/2007 |

## OTHER PUBLICATIONS

Japanese Office Action dated Apr. 19, 2011, issued in corresponding Japanese Patent Application No. 2007-022493.

\* cited by examiner

*Primary Examiner* — Mark Chapman

(74) *Attorney, Agent, or Firm* — Westerman, Hattori, Daniels & Adrian, LLP

(57) **ABSTRACT**

A toner for developing electrostatic image which has a reduced residual amount of a decomposed product of a polymerization initiator remaining in the toner upon production (mainly an ether component) and an unreacted polymerizable monomer (mainly styrene), less odor produced upon fixing so as to avoid deteriorating surrounding environment, an excellent shelf stability at high temperature upon storing or anti-blocking property, and an excellent printing durability under both N/N environment and H/H environment upon printing is provided. A toner for developing electrostatic image comprising a colored resin particle which is obtained by polymerizing a polymerizable monomer composition containing a polymerizable monomer, a colorant and a charge control resin in an aqueous dispersion medium in the presence of a polymerization initiator, wherein the charge control resin is a quaternary ammonium base containing copolymer having a glass transition temperature "Tg" in the range from 70 to 100°C.; the polymerization initiator is an organic peroxide; and each residual amount of an ether component and styrene remaining in the toner for developing electrostatic image is respectively less than 500 ppm and less than 50 ppm.

**19 Claims, 1 Drawing Sheet**



FIG. 1



## 1

**TONER FOR DEVELOPING  
ELECTROSTATIC IMAGE AND METHOD OF  
PRODUCING THE SAME**

**BACKGROUND OF THE INVENTION**

**1. Field of the Invention**

The present invention relates to a toner for developing electrostatic image used for development of a latent image of electrostatics in an electrophotography, an electrostatic recording method, an electrostatic printing process or the like. Particularly, the present invention relates to a toner for developing electrostatic image which has less odor produced upon fixing so as to avoid deteriorating surrounding environment and excellent printing durability. Hereinafter, "a toner for developing electrostatic image" may be simply referred to as "a toner".

**2. Description of the Related Art**

Image-forming devices such as an electrophotographic device, an electrostatic recording device, an electrostatic printing device and so on are applied to a copying machine, a printer, a facsimile machine, a complex machine thereof and so on. A method to form a desired image by developing a latent image of electrostatics formed on a photosensitive member with a toner for developing electrostatic image is widely used.

For example, an electrophotographic device using an electrophotography uniformly charges a surface of a photosensitive member generally formed of a photoconductive material with any means used generally, then, a latent image of electrostatics is formed on the photosensitive member. Next, the latent image of electrostatics is developed with the use of a toner. After transferring an image of the toner on a transferring material such as paper or the like, the image is fixed by a method such as heating or the like. Thus, a copy is obtained.

Conventionally, a toner produced by a pulverization method, which is a toner (pulverized toner) obtained by mixing and kneading a binder resin obtained by polymerizing a polymerizable monomer, a colorant and so on followed by pulverizing and classifying, has been generally used. However, the pulverization method has problems of decrease in yield, large energy consumption in pulverization and so on, particularly when producing a toner with a small particle diameter. In order to solve these problems, a toner produced by a polymerization method, a polymerized toner, has been proposed. The polymerized toner are likely to be small in diameter, have uniform form and have narrow size distribution, thus is excellent in printing performance in comparison with pulverized toner.

As a method of producing the polymerized toner, there may be a suspension polymerization method, an emulsion agglomeration method, a dispersion polymerization method and so on. For example, in the suspension polymerization method, firstly, a polymerizable monomer, a colorant, and if required, other additives are mixed to prepare a polymerizable monomer composition, and the polymerizable monomer composition is dispersed in an aqueous dispersion medium containing a dispersion stabilizer followed by agitation with a high-speed agitator or the like to form droplets of the polymerizable monomer composition. Next, the polymerizable monomer composition formed as the droplets is polymerized in the presence of a polymerization initiator followed by washing, filtering, dehydrating and drying, thus, colored resin particles are obtained. Further, the colored resin particles are mixed with an external additive such as an inorganic fine

## 2

particle or the like to obtain a polymerized toner. If required, the polymerized toner is mixed with a carrier to obtain a two-component developer.

In the above production process of the polymerized toner, some additives added as required disturb polymerization reaction of the polymerizable monomer. An unreacted polymerizable monomer remaining in the toner has been a problem. Also, besides the unreacted polymerizable monomer, it has been a problem that a decomposed product of a polymerization initiator is obtained as a by-product by polymerization using the polymerization initiator and remains in the toner.

If the unreacted polymerizable monomer and the decomposed product of the polymerization initiator remain in the toner, volatiles derived from the unreacted polymerizable monomer and the decomposed product of the polymerization initiator volatilize by heating upon fixing and odor is produced so that surrounding environment is deteriorated. Further, the toners become fusible each other upon storing the toner resulting in blocking, thus causing decrease in shelf stability of the toner and adverse effect on printing performance of the toner.

With respect to the above problem, production of odor upon fixing has been tried to be diminished. For example, Japanese Patent Application Laid-Open (JP-A) No. 2000-321809 suggests a method of producing a toner including a process of stripping treatment under reduced pressure (removal of unreacted polymerizable monomer) with a dispersion liquid containing a colored resin particle after suspension polymerization and discloses t-butylperoxy-2-ethylhexanoate (product name: PERBUTYL O; manufactured by NOF Corporation) as a polymerization initiator.

JP-A No. 2001-117272 suggests a method of producing a toner including a process of stripping treatment under reduced pressure (removal of unreacted polymerizable monomer) and a specific agitation condition with a dispersion liquid containing a colored resin particle after suspension polymerization and discloses t-butylperoxy-isobutyrate (product name: PERBUTYL IB; manufactured by NOF Corporation) as a polymerization initiator.

JP-A No. 2000-3076 suggests a method of producing a resin for toner obtained by copolymerizing styrene and (meth) acrylic acid ester using a polymerization initiator and discloses a group consisting of dicinnamoylperoxide and tertiary alkylperoxycinnamate having 4 to 8 carbons as a polymerization initiator.

JP-A No. 2000-321809 and JP-A No. 2001-117272 focus attention on the odor derived from an unreacted polymerizable monomer and try to reduce a residual amount of the unreacted polymerizable monomer remaining in a toner by a stripping treatment under reduced pressure. However, JP-A No. 2000-321809 and JP-A No. 2001-117272 do not focus attention on the odor derived from the decomposed product of the polymerization initiator and do not sufficiently solve the problem of odor. Also, a toner disclosed in JP-A No. 2000-3076 is a pulverized toner obtained by a pulverization method. Since a production process of the toner includes mixing and kneading at high temperature, a residual amount of an unreacted polymerizable monomer remaining in the toner is relatively small, thus odor derived from an unreacted polymerizable monomer produced is considered to be small. However, JP-A No. 2000-3076 does not try to diminish the decomposed product of the polymerization initiator used and the problem of odor is not sufficiently solved. Also, the remaining decomposed product of the polymerization initia-

tor not only produces the odor but also has effect on flowability and charging performance of toner, which causes decrease in printing durability of toner.

In addition to the problem of odor produced upon fixing, a toner is required to be excellent in printing durability so that the toner does not decline printing performance even in continuous printing of plural prints under a severe environment for using a toner such as a high temperature and humidity since use of toner in the area of high temperature and humidity is increasing in recent years. Also, a toner which is excellent in shelf stability at high temperature is required so that toners are not likely to be fusible each other even the toner is left or stored at high temperature.

As there has been such request, it has been necessary to design a toner in which change of charge amount due to environmental changes is small and which can keep a stable charge amount over time and such a toner has been discussed.

For example, JP-A No. Hei. 11 (1999)-15192 discloses a method of producing a toner wherein a polymerizable monomer is subject to suspension polymerization in a suspension medium containing a colorant and an inorganic dispersant in the presence of a quaternary ammonium base containing copolymer comprising a repeating structural unit derived from vinyl aromatic hydrocarbon, a repeating structural unit derived from (meth)acrylate and a repeating structural unit derived from quaternary ammonium base containing (meth)acrylate.

JP-A No. 11 (1999)-15192 is considered to be capable of obtaining a toner which is less likely to be fusible with other toners, can keep a stable charge amount over time to some extent and has shelf stability and printing durability been improved. However, in order to attain high-level requirement of recent years, it is considered that further study is necessary.

An object of the present invention is to provide a toner for developing electrostatic image which has a reduced residual amount of a decomposed product of a polymerization initiator remaining in the toner upon production (mainly an ether component) and an unreacted polymerizable monomer (mainly styrene), less odor produced upon fixing so as to avoid deteriorating surrounding environment, excellent shelf stability at high temperature upon storing or anti-blocking property, and excellent printing durability under both N/N environment and H/H environment upon printing.

#### SUMMARY OF THE INVENTION

As a result of diligent researches made to attain the above object, the inventor of the present invention found out that by obtaining a colored resin particle from polymerization in the presence of a specific polymerization initiator, a residual amount of a decomposed product of the polymerization initiator remaining in the toner upon production (mainly an ether component) and an unreacted polymerizable monomer (mainly styrene) can be reduced to be below a specific range, less odor is produced upon fixing, and by obtaining a colored resin particle from preparation of a polymerizable monomer composition with the use of a charge control resin having specific properties, change in charge amount due to environmental changes can be small, a charge amount can be stable over time, a shelf stability at high temperature upon storing or anti-blocking property is excellent, and a printing durability under both N/N environment and H/H environment upon printing can be improved, and completed the present invention based on the above knowledge.

A toner for developing electrostatic image of the present invention is a toner for developing electrostatic image comprising a colored resin particle which is obtained by polymer-

izing a polymerizable monomer composition containing a polymerizable monomer, a colorant and a charge control resin in an aqueous dispersion medium in the presence of a polymerization initiator,

wherein the charge control resin is a quaternary ammonium base containing copolymer having a glass transition temperature "Tg" in the range from 70 to 100° C.;

the polymerization initiator is an organic peroxide; and

10 each residual amount of an ether component and styrene remaining in the toner for developing electrostatic image is respectively less than 500 ppm and less than 50 ppm.

Also, a method of producing a toner for developing electrostatic image of the present invention is a method of producing a toner for developing electrostatic image comprising the steps of:

15 (1) a preparation process of a polymerizable monomer composition, in which a polymerizable monomer, a colorant, a quaternary ammonium base containing copolymer having a 20 glass transition temperature "Tg" in the range from 70 to 100° C. as a charge control resin are mixed together to prepare a polymerizable monomer composition;

25 (2) a suspension process, in which after the polymerizable monomer composition is dispersed in an aqueous dispersion medium comprising a dispersion stabilizer, an organic peroxide as a polymerization initiator is added and droplets of the polymerizable monomer composition are formed so as to obtain a suspension;

30 (3) a polymerization process, in which a temperature of the suspension is raised for polymerization so as to obtain an aqueous dispersion liquid of a colored resin particle; and

35 (4) a stripping process, in which the aqueous dispersion liquid of the colored resin particle is subject to a stripping treatment.

40 According to the toner for developing electrostatic image, a toner for developing electrostatic image which has a reduced residual amount of a decomposed product of a polymerization initiator remaining in the toner upon production (mainly an ether component) and an unreacted polymerizable monomer (mainly styrene), therefore, has less odor produced upon fixing so as to avoid deteriorating surrounding environment, an excellent shelf stability at high temperature upon storing or anti-blocking property, and an excellent printing durability under both N/N environment and H/H environment upon printing is provided.

#### BRIEF DESCRIPTION OF THE DRAWING

In the accompanying drawing,

50 FIG. 1 is a view showing a system used in a stripping treatment process employed in Examples of the present invention;

55 The numerical symbol in each FIGURE refers to the following: 1. an evaporator; 2. a jacket; 3. an agitator with stirring vane; 4. an aqueous dispersion of colored resin particles; 5. a gas blowing tube; 6. a blower; 7. a gas circulation line; 8. a condenser; 9. a condensation tank; 10. a gas circulation line; 11. a removal device for volatiles; 12. a gas circulation line; 13. a gas circulation line; and 14. a noncontact bubble level meter.

#### DETAILED DESCRIPTION OF THE INVENTION

60 A toner for developing electrostatic image of the present invention is a toner for developing electrostatic image comprising a colored resin particle which is obtained by polymerizing a polymerizable monomer composition containing a

polymerizable monomer, a colorant and a charge control resin in an aqueous dispersion medium in the presence of a polymerization initiator,

wherein the charge control resin is a quaternary ammonium base containing copolymer having a glass transition temperature "Tg" in the range from 70 to 100° C.;

the polymerization initiator is an organic peroxide; and

each residual amount of an ether component and styrene remaining in the toner for developing electrostatic image is respectively less than 500 ppm and less than 50 ppm.

Hereinafter, a toner for developing electrostatic image of the present invention and a production method thereof will be explained.

(1) Preparation Process of Polymerizable Monomer Composition

Firstly, a polymerizable monomer, a colorant, a charge control resin specified as in the present invention and other additives, if required, are mixed together to prepare a polymerizable monomer composition. A method of preparing the polymerizable monomer composition may not be particularly limited. For example, the polymerizable monomer composition can be prepared in such a manner that after the polymerizable monomer, the colorant and the charge control resin specified as in the present invention are agitated to mix by means of an agitator or the like, dispersion by means of a media type dispersing machine or the like is performed followed by adding, mixing and solving other additives, if necessary.

In the present invention, a polymerizable monomer means a compound which can be polymerized. As a main component of the polymerizable monomer, a monovinyl monomer is preferably used. As the monovinyl monomer, for example, there may be styrene; a styrene derivative such as vinyl toluene,  $\alpha$ -methylstyrene or the like; acrylic acid and methacrylic acid; acrylic acid ester such as methyl acrylate, ethyl acrylate, propyl acrylate, butyl acrylate, 2-ethyl hexyl acrylate, dimethylaminoethyl acrylate or the like; methacrylic acid ester such as methyl methacrylate, ethyl methacrylate, propyl methacrylate, butyl methacrylate, 2-ethyl hexyl methacrylate, dimethylaminoethyl methacrylate or the like; an amide compound such as acrylamide, methacrylamide or the like; olefin such as ethylene, propylene, butylene or the like; and so on. The monovinyl monomers may be used alone or in combination. Among them, styrene, a styrene derivative, an acrylic acid derivative or methacrylic acid derivative is suitably used as the monovinyl monomer. In the present invention, "(meth)acrylic acid" refers to "methacrylic acid and acrylic acid".

In order to prevent hot offset, as a part of the polymerizable monomer, any crosslinkable polymerizable monomer may be preferably used together with the monovinyl monomer. The crosslinkable polymerizable monomer means a monomer having two or more polymerizable functional groups. As the crosslinkable polymerizable monomer, for example, there may be an aromatic divinyl compound such as divinyl benzene, divinyl naphthalene, a derivative thereof or the like; unsaturated carboxylic acid polyester of polyalcohol such as ethylene glycol dimethacrylate, diethylene glycol dimethacrylate or the like; a divinyl compound other than the above such as N,N-divinylaniline, divinyl ether or the like; a compound having three or more vinyl groups such as trimethylolpropane trimethacrylate, dimethylolpropane tetraacrylate or the like; and so on. The crosslinkable polymerizable monomers may be used alone or in combination of two or more kinds.

In the present invention, the crosslinkable polymerizable monomers may be desirably used in an amount in the range of

generally from 0.1 to 5 parts by weight, preferably from 0.3 to 2 parts by weight, with respect to the monovinyl monomer of 100 parts by weight.

Further, as a part of the polymerizable monomer, any macromonomer may be preferably used together with the monovinyl monomer so that shelf stability and fixing ability at low temperature of the toner can be well-balanced. The macromonomer is a reactive oligomer or polymer which has a polymerizable carbon-carbon unsaturated double bond at the end of a polymer chain and a number average molecular weight of from 1,000 to 30,000 generally. As the macromonomer, a macromonomer which provides a polymer having higher "Tg" (glass transition temperature) than that of a polymer obtained by polymerization of the monovinyl monomer is preferable.

In the present invention, an amount of the macromonomer desirably used may be generally in the range from 0.01 to 10 parts by weight, preferably from 0.03 to 5 parts by weight, more preferably from 0.05 to 1 part by weight, with respect to the monovinyl monomer of 100 parts by weight.

A colorant is used in the present invention. To produce a colored toner, in which four types of toners including a black toner, a cyan toner, a yellow toner and a magenta toner are generally used, a black colorant, a cyan colorant, a yellow colorant and a magenta colorant may be respectively used.

In the present invention, as the black colorant, carbon black, titanium black, a magnetic powder such as zinc-ferric oxide, nickel-ferric oxide or the like may be used.

As the cyan colorant, for example, a compound such as a copper phthalocyanine pigment, a derivative thereof, an anthraquinone pigment or the like may be used. Specifically, there may be C. I. Pigment Blue 2, 3, 6, 15, 15:1, 15:2, 15:3, 15:4, 16, 17:1, 60 or the like. For good stability in polymerization and tinting strength of a toner obtained, the copper phthalocyanine pigment such as C. I. Pigment Blue 15, 15:1, 15:2, 15:3, 15:4, 17:1, or the like is preferable, and C. I. Pigment Blue 15:3 is more preferable.

As the yellow colorant, for example, a compound including an azo pigment such as a monoazo pigment, a disazo pigment or the like, a condensed polycyclic pigment and so on may be used. Specifically, there may be C. I. Pigment Yellow 3, 12, 13, 14, 15, 17, 62, 65, 73, 74, 83, 93, 97, 120, 138, 155, 180, 181, 185, 186 or the like.

As the magenta colorant, for example, a compound including an azo pigment such as a monoazo pigment, a disazo pigment or the like, a condensed polycyclic pigment and so on may be used. Specifically, there may be C. I. Pigment Red 31, 48, 57:1, 58, 60, 63, 64, 68, 81, 83, 87, 88, 89, 90, 112, 114, 122, 123, 144, 146, 149, 150, 163, 170, 184, 185, 187, 202, 206, 207, 209 or 251, C. I. Pigment Violet 19 or the like. For good stability in polymerization and tinting strength of a toner thus obtained, a monoazo pigment such as C. I. Pigment Red 31, 48, 57:1, 58, 60, 63, 64, 68, 112, 114, 146, 150, 163, 170, 185, 187, 206, 207 or the like may be preferable.

In the present invention, the colorants may be used alone or in combination of two or more kinds. An amount of the colorants desirably used may be preferably in the range from 1 to 10 parts by weight with respect to the monovinyl monomer of 100 parts by weight.

The charge control resin specified in the present invention is a quaternary ammonium base containing copolymer having a glass transition temperature "Tg" in the range from 70 to 100° C. The glass transition temperature "Tg" is preferably from 70 to 100° C., more preferably from 75 to 95° C. "Tg" is a value measured by Differential Scanning Calorimetry.

Since the quaternary ammonium base containing copolymer used as the charge control resin in the present invention is

high in compatibility with the polymerizable monomer in comparison with a conventionally used charge control agent, agitation and mixture with the polymerizable monomer, the colorant and other additive can be suitably performed. As the result, the quaternary ammonium base containing copolymer which is the charge control resin can be uniformly dispersed in the polymerizable monomer composition so as to prepare a desirable polymerizable monomer composition. If the glass transition temperature "Tg" is in the above range, a toner excellent in shelf stability at high temperature and printing durability under environment at high temperature and humidity since a balance between shelf stability and fixing ability of the toner can be taken and the toner can accommodate change in environment of storing and use.

Also, if the glass transition temperature "Tg" of the quaternary ammonium base containing copolymer used as the charge control resin in the present invention is below the above range, shelf stability of the toner may decline and printing performance of the toner may be adversely affected. On the other hand, if the glass transition temperature "Tg" of the quaternary ammonium base containing copolymer used as the charge control resin in the present invention exceeds the above range, fixing ability of the toner may decline and printing performance of the toner may be adversely affected.

Since the toner obtained by the desirable polymerizable monomer composition has a uniform charging ability over the whole particle, deterioration of charging ability is less likely to occur even if a continuous printing is performed with plural prints and printing performance such as fog or the like is less likely to decrease. Thus, such a toner is excellent in printing durability. Further, since the toner obtained by the desirable polymerizable monomer composition has small change in charge amount imparted to the toner particle even there is change in environment of storing and use and can maintain a stable charge amount over time, printing durability is excellent under environment at normal temperature and humidity and at high temperature and humidity. In the present invention, an NN environment refers to an environment with normal temperature and humidity based on a temperature of 23° C. and a humidity of 50%, and an HH environment refers to an environment with high temperature and humidity based on a temperature of 28° C. and a humidity of 80%.

The "quaternary ammonium base containing copolymer" used as the charge control resin in the present invention is preferably a copolymer comprising a repeating structural unit having quaternary ammonium base represented by the following Formula 2:

Formula 2:



wherein, R<sup>1</sup> is a hydrogen atom or a methyl group; R<sup>2</sup> is an alkylene group having 1 to 3 carbons; each of R<sup>3</sup> to R<sup>5</sup> is independently an alkyl group having 1 to 6 carbons, a phenyl group or an aralkyl group having 1 to 12 carbons; X is a halogen atom, an alkyl sulfonate residue having 1 to 6 carbons, a benzenesulfonate residue or a paratoluene sulfonate residue.

In the present invention, a vinyl monomer unit and a (meth)acrylate monomer unit may be preferably contained as the

repeating structural unit constituting the quaternary ammonium base containing copolymer besides the repeating structural unit having quaternary ammonium base represented by the Formula 2.

5 A containing amount of the repeating structural unit having quaternary ammonium base in the quaternary ammonium base containing copolymer is preferably in the range from 0.05 to 12 wt %, more preferably from 0.1 to 10 wt %. If the containing amount is within the above range, it is easier to control the charge amount of the quaternary ammonium base containing copolymer.

10 The quaternary ammonium base containing copolymer used as the charge control resin in the present invention may be produced, for example, by the following method:

- 15 1. a method to copolymerize the vinyl monomer and the quaternary ammonium base containing (meth)acrylate monomer;
2. a method to react the copolymer obtained in the above "1." with paratoluene sulfonate, methanesulfonic acid or the like; or
3. a method to quaternize a copolymer obtained by copolymerizing a vinyl monomer and a dialkylaminoalkyl (meth)acrylate monomer with a quaternization agent.

25 As examples of the quaternary ammonium base containing (meth)acrylate monomer, there may be N,N,N-trimethyl-N-(2-methacryloxyethyl)ammonium chloride (DMC: dimethylaminoethylmethyl methacrylate chloride), N-benzyl-N,N-dimethyl-N-(2-methacryloxyethyl)ammonium chloride (DML: dimethylaminoethylbenzyl methacrylate chloride) and so on.

30 As the dialkylaminoalkyl (meth)acrylate monomer, there may be dimethylaminoethyl (meth)acrylate, diethylaminoethyl (meth)acrylate, dipropylmethylaminoethyl (meth)acrylate, dibutylaminoethyl (meth)acrylate or the like.

35 As the quaternization agent, there may be a halogenated organic compound such as methyl chloride, methyl bromide, ethyl chloride, ethyl bromide, benzyl chloride, benzyl bromide or the like; sulfonate alkyl ester such as methyl sulfonate alkyl ester, ethyl sulfonate alkyl ester, propyl sulfonate alkyl ester, benzene sulfonate alkyl ester, paratoluene sulfonate alkyl ester or the like.

40 As the vinyl monomer, the vinyl aromatic hydrocarbon monomer and (meth)acrylate monomer mentioned in the above polymerizable monomer or the like is preferably used. As specific examples of the vinyl aromatic hydrocarbon monomer, there may be styrene, α-methylstyrene, 2-methylstyrene, 3-methylstyrene, 4-methylstyrene, 2-ethylstyrene, 3-ethylstyrene, 4-ethylstyrene, 2-propylstyrene, 3-propylstyrene, 4-propylstyrene, 2-isopropylstyrene, 3-isopropylstyrene, 4-isopropylstyrene, 2-chlorostyrene, 3-chlorostyrene,

45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 943

2-ethyl-3-methyl- $\alpha$ -methylstyrene, 2-methyl-4-propyl- $\alpha$ -methylstyrene, 2-chloro-4-ethyl- $\alpha$ -methylstyrene and so on.

As a specific example of the (meth) acrylic acid monomer, there may be a (meth)acrylate compound not having quaternary ammonium base (hereinafter, it may be simply referred to as a (meth)acrylate compound) such as acrylic acid ester including methyl acrylate, ethyl acrylate, propyl acrylate, isopropyl acrylate, n-butyl acrylate, isobutyl acrylate, n-amyl acrylate, isoamyl acrylate, n-hexyl acrylate, 2-ethylhexyl acrylate, hydroxypropyl acrylate, lauryl acrylate or the like; methacrylic acid ester including methyl methacrylate, ethyl methacrylate, propyl methacrylate, isopropyl methacrylate, n-butyl methacrylate, isobutyl methacrylate, n-amyl methacrylate, isoamyl methacrylate, n-hexyl methacrylate, 2-ethylhexyl methacrylate, hydroxypropyl methacrylate, lauryl methacrylate or the like.

In the case of containing the vinyl aromatic hydrocarbon monomer unit and the (meth)acrylate monomer unit as the repeating structural units constituting the quaternary ammonium base containing copolymer in the present invention, a copolymerization ratio (weight ratio) thereof may be preferably in the range from 70:30 to 90:10, more preferably from 75:25 to 88:12. If the copolymerization ratio is within the above range, it is easier to obtain the quaternary ammonium base containing copolymer having Tg specified in the present invention.

As the quaternary ammonium base containing copolymer used as the charge control resin in the present invention, various commercialized products may be used. As the commercialized product, for example, there may be FCA-592P (product name; manufactured by Fujikura Kasei Co., Ltd.; Tg: 82°C.; Mw: 12,000) or the like.

A weight average molecular weight "Mw" of the quaternary ammonium base containing copolymer used as the charge control resin in the present invention may be preferably in the range from 2,000 to 50,000, more preferably from 4,000 to 40,000, even more preferably from 6,000 to 35,000. If the weight average molecular weight "Mw" of the quaternary ammonium base containing copolymer used as the charge control resin in the present invention is within the above range, the quaternary ammonium base containing copolymer can be suitably dispersed in the polymerizable monomer composition, and can obtain a toner having a stable charge amount over time.

If the weight average molecular weight "Mw" of the quaternary ammonium base containing copolymer used as the charge control resin in the present invention is less than the above range, shelf stability or printing durability of the toner may decrease. On the other hand, if the weight average molecular weight "Mw" of the quaternary ammonium base containing copolymer used as the charge control resin in the present invention exceeds the above range, fixing ability of the toner may decrease.

An added amount of the quaternary ammonium base containing copolymer used as the charge control resin in the present invention may be preferably in the range from 0.01 to 20 parts by weight, more preferably from 0.3 to 10 parts by weight, with respect to 100 parts by weight of the binder resin. Herein, the standard of 100 parts by weight of the binder resin mentioned above is nearly equal to the standard of 100 parts by weight of the polymerizable monomer and can be substituted with 100 parts by weight of the polymerizable monomer.

If the added amount of the quaternary ammonium base containing copolymer used as the charge control resin in the present invention is within the above range, shelf stability at

high temperature when storing the toner and printing durability upon printing under the H/H environment can be effectively increased.

If the added amount of the quaternary ammonium base containing copolymer used as the charge control resin in the present invention is less than the above range, the charge amount imparted to the toner particle may be insufficient so that printing performance of the toner may be adversely affected. On the other hand, the added amount of the quaternary ammonium base containing copolymer used as the charge control resin in the present invention exceeds the above range, it may be difficult to control the charge amount and printing performance may lower.

As one of other additives, a release agent may be preferably added since it can improve a releasing characteristic of the toner from a fixing roller at fixing. As the release agent, one which is generally used as a release agent for the toner may be used without any particular limitation. There may be a polyolefin wax such as low-molecular-weight polyethylene, low-molecular-weight polypropylene, low-molecular-weight polybutylene or the like; a natural wax such as candelilla, a carnauba wax, a rice wax, a haze wax, jojoba or the like; a petroleum wax such as paraffin, microcrystalline, petrolac-tam or the like; a mineral wax such as montan, ceresin, ozokerite or the like; a synthesized wax such as a Fischer-Tropsch wax or the like; an esterified compound of polyalcohol including pentaerythritol ester such as pentaerythritol tetra-myristate, pentaerythritol tetrapalmitate, pentaerythritol tetrastearate, pentaerythritol tetralaurate or the like, dipentaerythritol ester such as dipentaerythritol hexamyrystate, dipentaerythritol hexopalmitate, dipentaerythritol hexylaurate or the like; and so on. Among them, the esterified compound of polyalcohol is preferable since it can improve the low-temperature fixing ability of the toner and cannot deteriorate printing durability. The esterified compounds may be used alone or in combination of two or more kinds.

In the present invention, an amount of the release agent desirably used may be generally in the range from 0.1 to 30 parts by weight, preferably from 1 to 20 parts by weight, with respect to the monovinyl monomer of 100 parts by weight.

As one of other additives, a molecular weight modifier may be preferably used. As the molecular weight modifier, there may be mercaptans such as t-dodecyl mercaptan, n-dodecyl mercaptan, n-octyl mercaptan, 2,2,4,6,6-pentamethylheptane-4-thiol or the like; thiuram disulfides such as tetramethyl thiuram disulfide, tetraethyl thiuram disulfide, tetrabutyl thiuram disulfide, N,N'-dimethyl-N,N'-diphenyl thiuram disulfide, N,N'-dioctadecyl-N,N'-disopropyl thiuram disulfidell or the like; and so on. The molecular weight modifier may be added prior to or during polymerization.

In the present invention, an amount of the molecular weight modifier desirably used may be generally in the range from 0.01 to 10 parts by weight, preferably from 0.1 to 5 parts by weight, with respect to the monovinyl monomer of 100 parts by weight.

## (2) Suspension Process of Obtaining Suspension (Droplets Forming Process)

The polymerizable monomer composition thus obtained in "(1) Preparation process of polymerizable monomer composition" is dispersed in an aqueous dispersion medium comprising a dispersion stabilizer. After addition of a polymerization initiator specified of the present invention, droplets of the polymerizable monomer composition are formed. If necessary, the molecular weight modifier and the cross-linkable polymerizable monomer may be added after the polymerization initiator specified in the present invention is added.

## 11

The timing of adding the polymerization initiator specified in the present invention may not be particularly limited. For instance, the polymerization initiator may be preliminarily added in the polymerizable monomer composition to form droplet. However, in the present invention, it is preferable that, as mentioned above, after the polymerizable monomer composition is dispersed in the aqueous dispersion medium containing the dispersion stabilizer and after forming droplets, the polymerization initiator specified in the present invention is added to form droplets.

The method of forming droplets may not be particularly limited. For example, droplets may be formed by means of a device capable of high dispersion such as MILDEN MDN303V (product name; manufactured by: Pacific Machinery & Engineering Co., Ltd.), MILDEN (product name; manufactured by Ebara Corporation) or the like as an in-line type emulsifying and dispersing machine, T. K. HOMOMIXER MARK II (product name; manufactured by PRIMIX Corporation) as a high-speed emulsification dispersing machine, CAVITRON CD 1000 (product name; manufactured by Pacific Machinery & Engineering Co., Ltd.) or the like.

The polymerization initiator specified in the present invention is organic peroxide. The organic peroxide used as the polymerization initiator in the present invention is a derivative of hydrogen peroxide ( $H-O-O-H$ ) having a structure in which one or two hydrogen atoms of hydrogen peroxide are substituted by organic atomic groups. Also, since a peroxidation bond ( $O-O$ ) of the organic peroxide has smaller bond energy than other bonds such as " $C-H$ ", " $C-C$ ", " $C-O$ " and so on, the peroxidation bond ( $O-O$ ) is easily decomposed (cleaved) by heating or the like and an oxygen radical ( $O$ ) of the organic peroxide is produced. The produced oxygen radical ( $O$ ) of the organic peroxide reacts with the polymerizable monomer to proceed the polymerization reaction.

The organic peroxide which is the polymerization initiator not only has effect to react with the polymerizable monomer due to decomposing (cleaving) of the peroxidation bond ( $O-O$ ) and proceed the polymerization reaction but also produces the decomposed product of the polymerization initiator (mainly an ether component) as by-product which remains in the toner to cause odor. Herein, the "ether component" which is a main component of the decomposed product of the polymerization initiator means a volatile ether component causing odor, specifically, a monoether component having one ether bond in one molecule of the decomposed product of the polymerization initiator but it does not include a polyether component having plural ether bonds in one molecule of the decomposed product of the polymerization initiator.

The above organic peroxide can be classified by chemical structure into seven kinds: a hydroperoxide compound (Formula 3), a dialkylperoxide compound (Formula 4), a peroxy ester compound (Formula 1, an alkylperester compound), a diacylperoxide compound (Formula 5), a peroxydicarbonate compound (Formula 6), a peroxyketal compound (Formula 7) and a ketone peroxide compound (Formula 8) represented by the following formulae,

Formula 3:



Formula 4:



## 12

-continued

Formula 1:



Formula 5:



Formula 6:



Formula 7:



Formula 8:



wherein, each of R, R', R'' may be an alkyl group or other organic group and may be the same or different with each other.

Among the above seven organic peroxides, the polymerization initiator used in the present invention is preferably the peroxy ester compound represented by the Formula 1 since the peroxy ester compound represented by the Formula 1 has a very high effect in decreasing residual amount of the decomposed product of the polymerization initiator (mainly ether component) and the unreacted polymerizable monomer (mainly styrene) remaining in the toner:

Formula 1:



wherein, each of R and R' is an alkyl group.

As the specific example of the peroxy ester compound preferably used as the polymerization initiator in the present invention, there may be t-butylperoxy-2-ethylbutanoate (product name: TRIGONOX 27 (Formula 9); manufactured by Akzo Nobel N.V.; molecular weight: 188; purity: 98%; one-hour half-life temperature: 94° C.), t-butylperoxy-2-ethylhexanoate (product name: PERBUTYL O (Formula 10); manufactured by NOF Corporation; molecular weight: 216; purity: 97%; one-hour half-life temperature: 92° C.), t-hexylperoxy-2-ethylhexanoate (product name: perhexyl O (Formula 11); manufactured by NOF Corporation; molecular weight: 244; purity: 90%; one-hour half-life temperature: 90° C.), 1,1,3,3-tetramethylbutylperoxy-2-ethylhexanoate (product name: perocta O (Formula 12); manufactured by NOF Corporation; molecular weight: 272; purity: 90%; one-hour half-life temperature: 84° C.), t-butylperoxy-pivalate (product name: perbutyl PV (Formula 13); manufactured by NOF Corporation; molecular weight: 174; purity: 70%; one-hour half-life temperature: 73° C.), t-hexylperoxy-pivalate (product name: perhexyl PV (Formula 14); manufactured by NOF Corporation; molecular weight: 202; purity: 70%; one-hour half-life temperature: 71° C.) represented by the following formulae or the like:

Formula 9:



Formula 10:



Formula 11:



Formula 12:



Formula 13:



Formula 14:



In the case of using the peroxy ester compound as the polymerization initiator in the present invention, a presumed structure of the by-produced decomposed product of the polymerization initiator may be, for example, a decomposed product represented by the following Formula 15 if TRIGO-NOX 27 (Formula 9) is used:

Formula 15:



Also, if PERBUTYL O (Formula 10) is used, a decomposed product represented by the following Formula 16 may be presumed:

Formula 16:



Further, carbon number of R and R' in the peroxy ester compound represented by the Formula 1 is preferably 6 or less, more preferably 5 or less. If the carbon number of R and

R' in the peroxy ester compound represented by the Formula 1 exceeds the above range, the boiling point of the decomposed product of the polymerization initiator becomes so high that it may be difficult to remove the decomposed product from the toner.

As the specific example of peroxy ester compound represented by Formula 1 in which carbon number of R and R' is 6 or less preferably used as the polymerization initiator in the present invention, there may be t-butylperoxy-2-ethylbutanoate (Formula 9), t-butylperoxy-pivalate (Formula 13), t-hexylperoxy-pivalate (Formula 14) or the like.

A molecular weight of the organic peroxide used as the polymerization initiator in the present invention is preferably 205 or less. If the molecular weight of the organic peroxide used as the polymerization initiator in the present invention is within the above range, since the molecular weight of the by-produced decomposed product of the polymerization initiator (mainly ether component) can be relatively small, the decomposed product of the polymerization initiator can be easily removed by performing the below mentioned stripping treatment with the colored resin particle having the decomposed product of the polymerization initiator remained.

If the molecular weight of the organic peroxide used as the polymerization initiator in the present invention exceeds the above range, since the molecular weight of the by-produced decomposed product of the polymerization initiator (mainly ether component) may be relatively large, it may be difficult to remove the decomposed product of the polymerization initiator even by performing the below mentioned stripping treatment with the colored resin particle having the decomposed product of the polymerization initiator remained.

A purity of the organic peroxide used as the polymerization initiator in the present invention is preferably 90% or more, more preferably 95% or more, even more preferably 97% or more. If the purity of the organic peroxide used as the polymerization initiator in the present invention is below the above range, impurity, diluent of the polymerization initiator and so on which are mixed upon producing the polymerization initiator may remain in the toner to decrease printing performance of the toner. Also, polymerization rate may decrease.

An one-hour half-life temperature of the organic peroxide used as the polymerization initiator of the present invention is preferably in the range from 70°C. to 100°C., more preferably from 75°C. to 95°C. The half life of the organic peroxide is a period of time when a concentration of the organic peroxide being a polymerization initiator is halved from an initial concentration. The half-life temperature is a temperature wherein a half life is one hour and is an indicator showing easiness of occurrence of the cleavage of the peroxidation bond (O—O) of the organic peroxide and produce radical.

If the one-hour half-life temperature of the organic peroxide used as the polymerization initiator in the present invention is below the above range, the polymerization rate may be higher so as to be difficult to control reaction. If the one-hour half-life temperature exceeds the above range, the polymerization rate may be lowered so as to take longer polymerization time.

An added amount of the organic peroxide used as the polymerization initiator in the present invention is preferably in the range from 0.1 to 15 parts by weight, more preferably from 0.5 to 10 parts by weight, even more preferably from 1 to 7 parts by weight, with respect to 100 parts by weight of the monovinyl monomer. If the added amount of the organic peroxide used as the polymerization initiator in the present invention is within the above range, a polymerization reaction mentioned hereinafter may be suitably performed and the

residual amounts of the decomposed product of the polymerization initiator (mainly ether component) and unreacted polymerizable monomer (mainly styrene) remained in the obtained colored resin particle can be decreased.

In the present invention, an aqueous dispersion medium may be water alone but a water-soluble solvent such as lower alcohol, lower ketone or the like may be used together. A dispersion stabilizer is preferably contained in the aqueous dispersion medium for use. As the dispersion stabilizer, for example, there may be a metallic compound and so on including sulfate such as barium sulfate, calcium sulfate or the like; carbonate such as barium carbonate, calcium carbonate, magnesium carbonate or the like; phosphate such as calcium phosphate or the like; metallic oxide such as aluminum oxide, titanium oxide or the like; metallic hydroxide such as aluminum hydroxide, magnesium hydroxide, ferric hydroxide or the like; and so on. As the dispersion stabilizer, there may be also an organic compound including a water-soluble polymer such as polyvinyl alcohol, methyl cellulose, gelatin or the like; an anionic surfactant; nonionic surfactant; an ampholytic surfactant; and so on. The dispersion stabilizer may be used alone or in combination of two or more kinds.

Among the dispersion stabilizer, the metallic compound, particularly, the dispersion stabilizer containing colloid of hardly water-soluble metal hydroxide is preferable since the particle distribution of the colored resin particle can be narrowed and the residual amount of the dispersion stabilizer remaining in the colored resin particle after washing can be small so that the polymerized toner to be obtained can reproduce clear image, particularly, image quality under the H/H environment is less likely to deteriorate.

### (3) Polymerization Process

A temperature of the desired suspension (the aqueous dispersion medium containing droplets of the polymerizable monomer composition) obtained in "(2) Suspension process of obtaining a suspension (droplets forming process)" is raised to polymerize in the presence of the polymerization initiator specified of the present invention.

In the present invention, polymerization temperature is preferably 50°C. or more, more preferably from 60 to 95°C. Polymerization reaction time is preferably from 1 to 20 hours, more preferably from 2 to 15 hours. In order to polymerize droplets of the polymerizable monomer composition in a state of being stably dispersed, the polymerization reaction may proceed while agitating the droplets for dispersion treatment in the polymerization process continuously following the "(2) Suspension process of obtaining suspension (droplets forming process)".

In the present invention, it is preferable to form so-called core-shell type (or "capsule type") colored resin particles, which can be obtained by using the colored resin particles obtained by the polymerization process as a core layer and forming a shell layer, a material of which is different from that of the core layer, around the core layer. The core-shell type colored resin particles can take a balance of lowering of fixing temperature and prevention of blocking at storage of a polymerized toner by covering the core layer comprising a substance having a low-softening point with a substance having a high softening point.

A method for producing the core-shell type colored resin particles mentioned above may not be particularly limited, and may be produced by a conventional method. An in situ polymerization method or a phase separation method is preferable from the viewpoint of production efficiency.

The method of producing the core-shell type colored resin particles according to the in situ polymerization method will be hereinafter described.

A polymerizable monomer (a polymerizable monomer for shell) for forming a shell layer and a polymerization initiator for shell are added to an aqueous dispersion medium to which the above-mentioned colored resin particles to be a core particle are dispersed followed by polymerization, thus the core-shell type colored resin particles can be obtained.

As a polymerizable monomer for shell, the above-mentioned polymerizable monomer or the like can be similarly used. Among them, a monomer which provides a polymer having "Tg" of more than 80°C. such as styrene, methyl methacrylate or the like may be preferably used alone or in combination of two or more kinds.

As a polymerization initiator for shell used for polymerization of the polymerizable monomer for shell, there may be polymerization initiators such as a metal persulfate including potassium persulfate, ammonium persulfate or the like; a water-soluble azo compound such as 2,2'-azobis-[2-methyl-N-(2-hydroxyethyl)propionamide], 2,2'-azobis-[2-methyl-N-(1,1-bis(hydroxymethyl)-2-hydroxyethyl)propionamide] or the like; and so on. In the present invention, an amount of the polymerization initiator for shell is preferably from 0.1 to 30 parts by weight, more preferably from 1 to 20 parts by weight with respect to the polymerizable monomer for shell of 100 parts by weight.

A polymerization temperature of the shell layer is preferably 50°C. or more, more preferably from 60 to 95°C. Also, the polymerization time of the shell layer is preferably in the range from 1 to 20 hours, more preferably from 2 to 15 hours.

### (4) Stripping Process

In the above "(3) Polymerization process", by using the polymerization initiator specified in the present invention, the polymerization reaction is suitably performed and the residual amount of the decomposed product of the polymerization initiator (mainly ether component) and unreacted polymerizable monomer (mainly styrene) remaining in the colored resin particle to be obtained can be decreased.

Further, in the present invention, if the decomposed product of the polymerization initiator (mainly ether component) and unreacted polymerizable monomer (mainly styrene) remain in the colored resin particle to be obtained even in small amount, it is preferable that the aqueous dispersion liquid of the colored resin particle obtained by the "(3) Polymerization process" is subject to the stripping treatment in order to efficiently remove volatiles (mainly ether component and styrene) which cause odor.

A stripping treatment system used in the present invention will be explained hereinafter.

As shown in FIG. 1, the stripping treatment system facilitates gas circulation lines (7, 10, 12 and 13) outside, and each gas circulation line comprises a blower 6, a condenser 8, a condensation tank 9 and a removal device for volatiles 11. An evaporator 1 of the stripping treatment system comprises an agitator 3 with stirring vane to agitate an aqueous dispersion 4 of colored resin particles inside of the evaporator 1. The evaporator 1 may be the same as the container (reactor) used in the polymerization process or may be different. On the outside of the evaporator 1, a jacket 2 for heating or cooling may be disposed.

Firstly, the aqueous dispersion liquid of the colored resin particle obtained by the "(3) Polymerization process" is diluted by the ion-exchange water so that the concentration of solid content of the colored resin particle is in the range from 10 to 30 wt %. An aqueous dispersion liquid 4 of the colored resin particle having the concentration of solid content adjusted is charged in the evaporator 1. If necessary, a defoaming agent is added in the evaporator 1. The stripping treatment is performed, heating is performed while stirring

with an agitator 3 with stirring vane and remaining volatiles remaining in the colored resin particles (mainly an ether component and styrene) can be removed.

As the stripping treatment, there may be a method of blowing gas to the aqueous dispersion 4 of colored resin particles; a method of blowing saturated vapor to the aqueous dispersion 4 of colored resin particles; and a method of depressurizing the aqueous dispersion 4 of colored resin particles. Among them, the method of blowing gas to the aqueous dispersion 4 of colored resin particles is preferable. When employing the method of blowing gas, the gas includes nitrogen, an inert gas of carbon dioxide or the like, air and so on. Among them, nitrogen is preferable. The gas may be blown to a gas phase part of the evaporator 1 (onto the surface of the aqueous dispersion 4 of colored resin particles). However, it is preferable to blow the gas into the aqueous dispersion 4 of colored resin particles.

After completing the stripping treatment, foam formation is likely to occur on the surface of the aqueous dispersion 4 of colored resin particles. If forms are overproduced and the aqueous dispersion 4 of colored resin particles spills from the evaporator 1, it flows into the gas circulation line 7 so as to contaminate. For this reason, it is preferable to use a defoaming agent with an effect of inhibiting foam formation. As the defoaming agent, there may be a fatty oil-based defoaming agent, a mineral oil-based defoaming agent, a polyether defoaming agent, a polyalkylene glycol-contained nonionic surfactant or the like. An amount of the defoaming agent to be added is preferably from 0.01 to 1 part by weight, more preferably from 0.05 to 0.5 parts by weight with respect to the colored resin particle of 100 parts by weight.

In order to remove remaining volatiles remaining in the colored resin particles (mainly ether component and styrene) by using the stripping treatment system, a temperature of the stripping treatment is preferably a glass transition temperature (Tg) of a binder resin comprising the colored resin particles or more and less than  $(Tg+75)^\circ C$ ., more preferably  $(Tg+10)^\circ C$ . or more and less than  $(Tg+65)^\circ C$ .

Time required for the stripping treatment may be appropriately determined depending on the scale of a stripping treatment system (treatment ability) and amounts of volatiles remaining in the colored resin particles (mainly ether component and styrene). Time required for the stripping treatment may be preferably in the range from 0.5 to 40 hours, more preferably from 1 to 20 hours.

In the stripping treatment system, if the temperature and time for the stripping treatment are in the above range, the volatiles remaining in the colored resin particles (mainly ether component and styrene) can be efficiently removed.

#### (5) Processes of Washing, Filtering, Dehydrating and Drying

It is preferable that the aqueous dispersion of colored resin particles obtained after the stripping process (4) is subject to a series of operations including washing, filtering, dehydrating, and drying several times as needed according to a conventional method.

Firstly, in order to remove the dispersion stabilizer remained in the aqueous dispersion of colored resin particles, acid or alkali is added to the aqueous dispersion to wash. If the dispersion stabilizer is an acid-soluble inorganic compound, acid is added to the aqueous dispersion of colored resin particles. On the other hand, if the dispersion stabilizer is an alkali-soluble inorganic compound, alkali is added to the aqueous dispersion of colored resin particles.

When using an acid-soluble inorganic compound as the dispersion stabilizer, it is preferable to control pH of the aqueous dispersion of colored resin particles to 6.5 or less by adding acid. It is more preferable to control pH to 6 or less. As

the acid to be added, an inorganic acid such as a sulfuric acid, a hydrochloric acid, a nitric acid or the like, or an organic acid such as a formic acid, acetic acid or the like may be used. Among them, the sulfuric acid is particularly preferable for high removal efficiency and small impact on production facilities.

After the above acid or alkali washing, a washing treatment (washing, filtering and dewatering) is performed using cleaning water such as ion-exchange water or the like followed by a drying treatment. As methods of washing, various known methods can be used and may not be particularly limited. For example, there may be a centrifugal filtration, a pressure filtration, a vacuum filtration or the like. As a washing device, a peeler centrifuge, a siphon peeler centrifuge or the like may be used for the washing treatment (washing, filtering and dehydrating). A method of drying may not be particularly limited also, and various known methods can be used. For example, various methods such as vacuum drying, flash drying, a spray dryer and so on may be used.

#### (6) Colored Resin Particles

The residual amount of the decomposed product of the polymerization initiator (mainly ether component) and unreacted polymerizable monomer (mainly styrene) remaining in the colored resin particle obtained by the above "(5) Processes of washing, filtering, dehydrating and drying" can be very small and odor derived from volatiles (mainly ether component and styrene) is produced very little upon printing using the obtained toner.

The colored resin particle comprising the toner will be hereinafter described. Hereinafter, the colored resin particle includes both core-shell type colored resin particle and colored resin particle which are not core-shell type.

A volume average particle diameter "Dv" of the colored resin particles comprising the toner for developing an electrostatic image of the present invention may be preferably in the range from 3 to 15  $\mu m$ , more preferably from 4 to 12  $\mu m$ . If "Dv" is less than the above range, flowability of the toner lowers, transferability of the toner may deteriorate, blur may generate, or printing density may lower. If "Dv" exceeds the above range, resolution of an image to be obtained may decline.

In the present invention, a number percentage of particle diameter of the colored resin particle of 5  $\mu m$  or less is preferably 25% or less, more preferably 18% or less. If the number percentage of particle diameter of the colored resin particle of 5  $\mu m$  or less exceeds the above range, flowability of the toner to be obtained may decrease, transferability of the toner may deteriorate. As a result, blur may generate and printing density may decline.

As for the colored resin particles in the present invention, a size distribution, which is a ratio "Dv/Dp" of a volume average particle diameter "Dv" and a number average particle size "Dp", may be preferably in the range from 1.0 to 1.3, more preferably from 1.0 to 1.2. If the size distribution "Dv/Dp" of the colored resin particles in the present invention exceeds the above range, flowability of the toner to be obtained lowers, transferability may decline; blur may generate, printing density may decline. The volume average particle diameter "Dv" and the number average particle size "Dp" of the colored resin particles may be measured, for example, by means of a particle diameter measuring device (product name: MULTISIZER; manufactured by Beckman Coulter, Inc.) or the like.

An average circularity of the colored resin particles in the present invention is preferably in the range from 0.960 to 0.995, more preferably from 0.970 to 0.995. In the present invention, circularity is a value obtained by dividing a perimeter of a circle having an area same as a projected image of a

particle by a perimeter of a particle image. Also, in the present invention, an average circularity is used as a simple method of presenting a shape of a particle quantitatively and is an indicator showing the level of convexo-concave shapes of the colored resin particle. The average circularity is "1" when the colored resin particles is an absolute sphere, and becomes smaller as the shape of the surface of the colored resin particles becomes more complex. In order to obtain the average circularity (Ca), firstly, circularity (Ci) of each of measured "n" particles of 0.6 µm or more by a diameter of the equivalent circle is calculated by the following Calculation formula 1. Next, the average circularity (Ca) is obtained by the following Calculation formula 2.

Calculation Formula 1:

circularity (Ci)=a perimeter of a circle having an area same as a projected area of a particle image/a perimeter of a particle image

$$Ca = \frac{\sum_{i=1}^n (Ci \times fi)}{\sum_{i=1}^n (fi)} \quad \text{Calculation formula 2}$$

In the Calculation formula 2, "fi" is a frequency of a particle of circularity (Ci).

The above-mentioned circularity and average circularity may be measured by means of a flow particle image analyzer FPIA-2000, FPIA-2100 or FPIA-3000 (product name; manufactured by Sysmex Co.) or the like.

If the average circularity of the colored resin particles exceeds the above range, the colored resin particles can easily pass through between a cleaning blade and a photosensitive member so that cleaning problems such as filming on the photosensitive member or fog of printed image is likely to occur. If the average circularity of the colored resin particles is less than the above range, reproducibility of thin lines may decrease.

The colored resin particles obtained in the present invention may be a toner for developing an electrostatic image as it is or a toner for developing an electrostatic image by adding carrier particles (ferrite, iron powder or the like). Also, the colored resin particles and an external additive may be mixed by means of a high-speed agitator such as HENSCHEL MIXER (product name; manufactured by: Mitsui Mining Co., Ltd.) or the like to form a one-component toner in order to control charge property, flowability, shelf stability or the like of a toner. Further, in addition to the colored resin particles and the external additive, carrier particles may be mixed to form a two-component developer.

As the external additive, there may be inorganic microparticles such as silica, titanium oxide, aluminum oxide, zinc oxide, tin oxide, calcium carbonate, calcium phosphate, cerium oxide or the like; and organic microparticles comprising a polymethyl methacrylate resin, silicone resin, melamine resin or the like. Among them, the inorganic microparticles are preferable. Silica and titanium oxide are more preferable, and silica is still more preferable. Further, as the external additive, two or more kinds of microparticles may be preferably used in combination. In the present invention, an amount of the external additive desired to be used is generally in the range from 0.1 to 6 parts by weight, preferably from 0.2 to 5 parts by weight, with respect to the colored resin particles of 100 parts by weight.

(7) Toner

The toner obtained through the above steps from (1) to (6) is obtained through the preparation of the polymerizable monomer composition using the charge control resin having specific characteristics, a suitable polymerization reaction using a specific polymerization initiator, and preferably the stripping treatment. Therefore, the residual amount of the decomposed product of the polymerization initiator (mainly ether component) and unreacted polymerizable monomer (mainly styrene) remaining in the toner can be lowered below a specific amount.

In the present invention, it is preferable that a residual amount of the ether component remaining in the toner is less than 500 ppm, preferably less than 200 ppm, more preferably less than 50 ppm. If the residual amount of the ether component remaining in the toner is in the above range, odor derived from the decomposed product of the polymerization initiator (mainly ether component) produced upon fixing can be decreased in very small amount so that the surrounding environment is not deteriorated.

It is preferable that the residual amount of styrene remaining in the toner of the present invention is less than 50 ppm, more preferably less than 30 ppm, even more preferably less than 20 ppm. If the residual amount of styrene remaining in the toner is within the above range, the odor derived from unreacted polymerizable monomer (mainly styrene) produced upon fixing can be reduced to a very small amount, surrounding environment may not be deteriorated, toners are less likely to be fusible with each other upon storage and shelf stability at high temperature (anti-blocking property) can be excellent.

Since the toner of the present invention is obtained by the suitable polymerization reaction using the specific polymerization initiator and preferably by the stripping treatment, the residual amount of the decomposed product of the polymerization initiator (mainly ether component) and unreacted polymerizable monomer (mainly styrene) remaining in the toner causing odor produced at fixing can be reduced below the specific amount, the toner of the present invention is a toner which does not deteriorate surrounding environment and takes environment into account.

Also, since the toner of the present invention is obtained by preparing the polymerizable monomer composition using the charge control resin having the specific properties, change of charge amount due to environmental changes is small, a stable charge amount can be maintained over time, shelf stability at high temperature (anti-blocking property) is excellent at storage, deterioration of image due to fog or the like is less likely to occur upon continuous printing of plural prints not only under the N/N environment at printing but also under the H/H environment (printing durability is excellent). Therefore, the toner of the present invention is a toner which meets the requirement of increased variation of storage environments and using environments of the toner and the requirement of decrease in printing cost.

## EXAMPLES

Hereinafter, the present invention will be explained further in detail with reference to examples and comparative examples. However, the scope of the present invention may not be limited to the following examples. Herein, "part(s)" and "%" are based on weight if not particularly mentioned. Test methods used in the examples and the comparative examples are as follows.

(1) Glass Transition Temperature

About 10 mg of test sample (a charge control resin) was weighed and, in accordance with ASTM D3418-97 using a

Differential Scanning Calorimetry (product name: SSC5200; manufactured by: Seiko Instruments, Inc.), charged into an aluminum pan. Measurement of the glass transition temperature ( $T_g$ ) of the test sample (the charge control resin) was performed using an empty aluminum pan as a reference under the condition of the temperature in the range from 0 to 150°C. and a heating rate of 10°C./min.

(2) Particle Diameter of Colored Resin Particle

The volume average particle diameter “ $D_v$ ” and the number average particle diameter “ $D_p$ ” of the colored resin particle were measured by means of a particle diameter measuring device (product name: MULTISIZER; manufactured by: Beckman Coulter, Inc.). Measurement by means of MULTISIZER was carried out under the condition of an aperture diameter of 100  $\mu\text{m}$ , using ISOTON II (product name; manufactured by Beckman Coulter, Inc.) as a medium, and a number of the measured particles of 100,000. More specifically, a colored resin particle sample of 0.2 g was charged into a beaker adding an aqueous solution of alkyl benzene sulfonate (product name: DRIWEL; manufactured by: Fuji film Corporation) of 0.5 ml as a dispersing agent. Further, 2 ml of the medium was added to the beaker to moist the colored resin particle. 10 ml of the medium was added. The mixture was dispersed by means of an ultrasonic disperser for 1 minute and was subject to measurement by means of the above particle diameter measuring device.

(3) Residual Amounts of Ether Component and Styrene

The toner was precisely weighed to be 3 g up to the unit of 1 mg. 27 g of ethyl acetate was added to the weighed toner of 3 g and agitated for 15 minutes. Then, 13 g of methanol was added thereto and agitated for another 10 minutes. A solution thus obtained was left to precipitate insoluble contents. A supernatant liquid of the solution was taken as a measurement sample and 2  $\mu\text{l}$  thereof was charged into a gas chromatograph to quantitate an ether component and styrene.

Measurement conditions of the gas chromatograph are as follows. A column (product name: DB-5; manufactured by: Agilent Technologies) with an inside diameter of 0.25 mm and a length of 30 m was used. The column was kept at 40°C. for three minutes. Then, the temperature was increased to 130°C. at a pace of 10°C. per minute and further increased to 230°C. at a pace of 20°C. per minute so that an injection temperature was 200°C. and a FID detection temperature was 250°C. As a standard sample for quantitative determination, an ethyl acetate/methanol solution of each component was used.

(4) Evaluation of Shelf Stability at High Temperature

A container charged with a toner of 20 g was hermetically closed and sunk in a constant temperature water bath kept at 60°C. The container was removed therefrom after five hours. The toner was transferred from the container onto a 42 mesh screen while being kept from vibration and set on a powder characteristics measuring device (product name: POWDER CHARACTERISTICS TESTER PT-R; manufactured by: Hosokawa Micron Corporation). The screen was vibrated at amplitude of 1.0 mm for 30 seconds. A weight of the toner remained on the screen was measured and referred to as a weight of the aggregated toner. Shelf stability rate (%) of the toner at high temperature was calculated from the ratio (% by weight) of the weight of the toner remained on the screen (corresponding to the weight of the aggregated toner) with respect to the weight of the toner measured (20 g). As the value of the shelf stability rate (%) of the toner at high temperature becomes smaller, the toner is less aggregated and more excellent in shelf stability at high temperature.

(5) Continuous Printing Test (N/N Environment, H/H Environment)

A commercially available printer of a non-magnetic one-component developing method (printing speed: 22 prints per minute) was charged with printing papers and inserted with a cartridge charged with a toner. After the printer was left under a N/N (normal temperature and humidity) environment having a temperature of 23°C. and a humidity of 50% for one day, continuous printing with 1% printing density was performed under the N/N environment. A solid patterned image with 0% image density was printed every 1,000 prints to measure a fog value. Number of sheets was counted while the image quality having the fog value of 1.0 or less is maintained when solid patterned images with 0% printing density were printed. The continuous printing test was performed up to 20,000 sheets but when fog is generated in mid-course, the continuous printing test was stopped at the time.

The fog value was measured as follows. After solid pattern printing with 0% image density of the first page was performed with the printer followed by stopping solid pattern printing at the tenth page, the toner of a nonimage area remained on the photosensitive member after developing was attached to an adhesive tape (product name: SCOTCH MENDING TAPE 810-3-18; manufactured by: Sumitomo 3M Limited). The tape was attached to a new printing paper, and color tone was measured by means of a spectrophotometer (product name: SE-2000; manufactured by: NIPPON DENSHOKU INDUSTRIES CO., LTD.). As a reference (or a benchmark sample), an unused tape was attached to a printing paper so as to measure a color tone in the same manner. Each color tone was referred as a coordinate of  $L^*a^*b^*$  space, and color difference  $\Delta E$  was calculated from the color tones of the sample for measurement and the benchmark sample. The color difference  $\Delta E$  is called a fog value. As the fog value decreases, less fog is produced and image quality is excellent.

The similar continuous printing test was performed under a H/H (high temperature and humidity) environment having a temperature of 28°C. and a humidity of 80%.

(6) Odor Evaluation

An odor evaluation of toner was performed in the following manner. 10 monitors were randomly selected. The monitors were allowed to judge an odor of a source of vacuum of the printer after printing 1,000 prints in the above continuous printing test (N/N environment). Evaluation was presented by the following criteria:

- A: 9 or more out of 10 monitors found the odor not uncomfortable;
- B: from 6 to 8 out of 10 monitors found the odor not uncomfortable; and
- C: 5 or more out of 10 monitors found the odor uncomfortable.

Example 1

75 parts of styrene and 25 parts of n-butyl acrylate as monovinyl monomers (calculated  $T_g$  of copolymer to be obtained=44°C.), 5 parts of a copper phthalocyanine pigment (C. I. Pigment Blue 15:3) as a cyan colorant, 1 part of quaternary ammonium base containing copolymer (a styrene/acrylic resin having 2 wt % of a quaternary ammonium base containing (meth)acrylate monomer unit; product name: FCA-592P; manufactured by: Fujikura Kasei Co., Ltd.;  $T_g$ : 82°C.;  $M_w$ : 12,000) as a charge control resin and 0.25 parts of polymethacrylic acid ester macromonomer (product name: AA6; manufactured by Toagosei Co., Ltd.;  $T_g$ =94°C.) were agitated by means of an agitator to mix followed by uniform dispersion by a media type dispersing machine. Thereto, 5 parts of dipentaerythritol hexamyrystate (solubility against styrene: 10 g/100 g or more; endothermic peak temperature: 65°C.; molecular weight: 1,514) as a release agent was added, mixed and solved, thus obtained a polymerizable monomer composition.

Separately, an aqueous solution of 4.8 parts of sodium hydroxide (alkali hydroxide metal) dissolved in 50 parts of ion-exchanged water was gradually added to an aqueous solution of 8.6 parts of magnesium chloride (water-soluble polyvalent metallic salt) dissolved in 250 parts of ion-exchanged water while agitating to prepare a magnesium hydroxide colloid (hardly water-soluble metal hydroxide colloid) dispersion liquid. A particle size distribution of the magnesium hydroxide colloid obtained was measured by means of a particle diameter measuring device (product name: SALD; manufactured by Shimadzu Corporation). The particle diameter of D50 (50% cumulative value of number particle size distribution) was 0.36  $\mu\text{m}$  and the particle diameter of D90 (90% cumulative value of number particle size distribution) was 0.80  $\mu\text{m}$ .

The polymerizable monomer composition was charged into the magnesium hydroxide colloid dispersion liquid thus obtained and agitated at room temperature until droplets are stable. Then, 5 parts of t-butylperoxy-2-ethylbutanoate represented by the following Formula 9 (product name: TRIGONOX 27; manufactured by: Akzo Nobel N.V.; purity: 98%; molecular weight: 188; one-hour half-life temperature: 94° C.) as a polymerization initiator, 1.2 parts of t-dodecyl mercaptan as a molecular weight modifier and 0.5 part of divinyl benzene as a cross-linking polymerizable monomer were added therein. The mixture was subject to a high shear agitation at 15,000 rpm for 10 minutes by means of an in-line type emulsifying and dispersing machine (product name: EBARA MILDERR; manufactured by Ebara Corporation) to form droplets of the polymerizable monomer composition.

Formula 9:



A thus obtained suspension having droplets of the polymerizable monomer composition dispersed (a polymerizable monomer composition dispersion liquid) was charged into a reactor furnished with a stirring vane and a temperature thereof was raised to 90° C. to start a polymerization reaction. When a polymerization conversion rate reached 95%, 1 part of methyl methacrylate as a polymerizable monomer for shell and 0.1 part of 2,2'-azobis-[2-methyl-N-(1,1-bis(hydroxymethyl)-2-hydroxyethyl)propionamide] (product name: VA-086; manufactured by: Wako Pure Chemical Industries, Ltd.) dissolved in 10 parts of ion-exchanged water as a polymerization initiator for shell were added to the suspension. After continuing the reaction for three hours at 90° C., the reaction was stopped to obtain an aqueous dispersion of colored resin particles having a core-shell structure having pH of 9.5.

The aqueous dispersion of colored resin particles thus obtained was subject to the following stripping treatment by means of a stripping treatment system shown in FIG. 1 and by a method of blowing gas as a stripping process.

Firstly, the aqueous dispersion 4 of colored resin particles was diluted with ion-exchanged water to have a solid density of 20% and supplied to an evaporator 1. Next, 0.1 part of a defoaming agent (product name: SN DEFOAMER 180; manufactured by: San Nopco Limited) was added to the evaporator 1. A nitrogen gas was run into the evaporator 1, and a gas phase part in the evaporator was substituted with the nitrogen gas.

After the aqueous dispersion of colored resin particles was heated to 80° C. while agitating by means of agitator 3 with the stirring vane 3, a blower 6 was activated to control a flow rate of the nitrogen gas to 0.6  $\text{m}^3/(\text{hr}\cdot\text{kg})$ . The nitrogen gas was blown in the aqueous dispersion of colored resin particles through a gas blowing tube 5, a gas outlet of which has a straight tube shape, to remove volatiles from the colored resin particle.

The nitrogen gas after stripping was directed to a condenser 8 and a condensation tank 9 in this order through a gas circulation line 7. The nitrogen gas after condensation was directed to a removal device for volatiles 11 (an absorption tower filled with activated carbon) through a gas circulation line 10 to remove volatiles contained in the nitrogen gas. The nitrogen gas, which no longer contains volatiles, was blown to the evaporator 1 again through a gas circulation line 12, the blower 6 and then a gas circulation line 13.

The stripping treatment was performed for six hours at a temperature of the aqueous dispersion of colored resin particles of 80° C., a pressure in the evaporator 1 of 101 kPa and a flow rate of the nitrogen gas of 0.6  $\text{m}^3/(\text{hr}\cdot\text{kg})$ . After the treatment for six hours, the aqueous dispersion of colored resin particles was cooled down to room temperature.

Thereafter, the aqueous dispersion of colored resin particles was subject to acid washing in which sulfuric acid was added to be pH of 6.5 or less while agitating at room temperature. After separating water by filtration, the aqueous dispersion of colored resin particles was subject to water washing in which another 500 parts of ion-exchanged water was added to make a slurry again. After repeating a series of dewatering and water washing several times, the colored resin particles were separated by filtration and charged into a container of a vacuum dryer for vacuum drying at 30 torr pressure and 50° C. for one day.

The volume average particle diameter "Dv" of the colored resin particles obtained was 9.5  $\mu\text{m}$ , and the size distribution "Dv/Dp" was 1.16. A thickness of shell calculated from the amount of polymerizable monomer for shell and a particle diameter of core particle (colored resin particle before forming the shell) was 0.03  $\mu\text{m}$  and sphericity "Sc/Sr" was 1.2.

To the colored resin particles thus obtained of 100 parts, silica particles subjected to a hydrophobicity-imparting treatment (product name: TG820F; manufactured by: Cabot Corporation) of 0.8 part and silica particles subjected to a hydrophobicity-imparting treatment (product name: NA50Y; manufactured by: Nippon Aerosil Co., Ltd.) of 1.0 part were added and mixed by means of a high speed agitator (product name: HENSCHEL MIXER; manufactured by Mitsui Mining Co., Ltd.) to produce a non-magnetic one-component toner of Example 1 for testing.

## Example 2

A toner of Example 2 was produced similarly as Example 1 except that the polymerization initiator was changed to t-butylperoxy-2-ethylhexanoate represented by the following Formula 10 (product name: PERBUTYL O; manufactured by NOF Corporation; molecular weight: 216; purity: 97%; one-hour half-life temperature: 92° C.), the stripping time was changed to 85° C. and the stripping time was changed to 10 hours:

Formula 10:



Similar tests as Example 1 were conducted with the toner of Example 2.

## Comparative Example 1

A toner of Comparative example 1 was produced similarly as Example 1 except that the charge control resin was changed to a quaternary ammonium base containing copolymer (styrene/acrylic resin; product name: FCA-207P; manufactured by Fujikura Kasei Co., Ltd.; Tg: 64° C.). Similar tests as Example 1 were conducted with the toner of Comparative example 1.

## Comparative Example 2

A toner of Comparative example 2 was produced similarly as Example 2 except that the charge control resin was changed to a quaternary ammonium base containing copolymer (styrene/acrylic resin; product name: FCA-207P; manufactured by Fujikura Kasei Co., Ltd.; Tg: 64° C.). Similar tests as Example 2 were conducted with the toner of Comparative example 2.

## Comparative Example 3

A toner of Comparative example 3 was produced similarly as Example 1 except that the polymerization initiator was changed to t-butyperoxy-2-ethylhexanoate represented by the above-mentioned Formula 10 (product name: PERBUTYL O; manufactured by NOF Corporation; molecular weight: 216; purity: 97%; one-hour half-life temperature: 92° C.) and the amount of the polymerization initiator was changed to 6 parts. Similar tests as Example 1 were conducted with the toner of Comparative example 3.

## &lt;Results&gt;

The test results of Examples and Comparative examples are shown in Table 1.

vironments since Comparative example 1 and Comparative example 2 did not use the quaternary ammonium base containing copolymer specified of present invention as the charge control resin.

Also, Comparative example 3 used the quaternary ammonium base containing copolymer specified of present invention as the charge control resin of the toner. However, since the residual amount of the ether component exceeded the range specified in the present invention, the toner of Comparative example 3 was inferior in shelf stability at high temperature and inferior in printing durability under the N/N and H/H environments.

To the contrary, Example 1 and Example 2 used the quaternary ammonium base containing copolymer (FCA-592P) specified of the present invention as the charge control resin of the toner. Hence, the toners of Example 1 and Example 2 were small in residual amount of ether component and styrene remaining in toner, were small in odor generation, were excellent in shelf stability at high temperature, could stably hold charge amount of toner and were excellent in printing durability under the N/N and H/H environments.

## What is claimed is:

1. A toner for developing electrostatic image comprising a colored resin particle which is obtained by polymerizing a polymerizable monomer composition containing a polymerizable monomer, a colorant and a charge control resin in an aqueous dispersion medium in the presence of a polymerization initiator,

wherein the charge control resin is a quaternary ammonium base containing copolymer having a glass transition temperature "Tg" in the range from 75 to 95° C.;

TABLE 1

|                               |                                                  | Example 1                                              | Example 2                                              | Comparative example 1                                  | Comparative example 2                                  | Comparative example 3                                  |
|-------------------------------|--------------------------------------------------|--------------------------------------------------------|--------------------------------------------------------|--------------------------------------------------------|--------------------------------------------------------|--------------------------------------------------------|
| Charge control resin          | Resin                                            | Quaternary ammonium base containing copolymer FCA-592P | Quaternary ammonium base containing copolymer FCA-592P | Quaternary ammonium base containing copolymer FCA-207P | Quaternary ammonium base containing copolymer FCA-207P | Quaternary ammonium base containing copolymer FCA-592P |
|                               | Product name                                     |                                                        |                                                        |                                                        |                                                        |                                                        |
|                               | Tg (° C.)                                        | 82                                                     | 82                                                     | 64                                                     | 64                                                     | 82                                                     |
|                               | Added amount (part by wt)                        | 1                                                      | Same as Example 1                                      | Same as Example 1                                      | Same as Example 2                                      | Same as Example 1                                      |
| Polymerization initiator      | Chemical name                                    | t-butyperoxy-2-ethylbutanoate                          | t-butyperoxy-2-ethylhexanoate                          | t-butyperoxy-2-ethylbutanoate                          | t-butyperoxy-2-ethylhexanoate                          | t-butyperoxy-2-ethylhexanoate                          |
|                               | Product name                                     | TRIGONOX 27                                            | PERBUTYL 0                                             | TRIGONOX 27                                            | PERBUTYL 0                                             | PERBUTYL 0                                             |
|                               | Added amount (part by wt)                        | 5                                                      | Same as Example 1                                      | Same as Example 1                                      | Same as Example 2                                      | 6                                                      |
| Molecular weight modifier     | Chemical name                                    | t-dodecyl mercaptan                                    | Same as Example 1                                      | Same as Example 1                                      | Same as Example 2                                      | Same as Example 1                                      |
|                               | Added amount (part by wt)                        | 1.2                                                    | Same as Example 1                                      | Same as Example 1                                      | Same as Example 2                                      | Same as Example 1                                      |
| Stripping treatment           | Temperature (° C.)                               | 80                                                     | 85                                                     | 80                                                     | 85                                                     | 80                                                     |
| Residual component in toner   | Time (hr)                                        | 6                                                      | 10                                                     | 6                                                      | 10                                                     | 6                                                      |
|                               | Residual amount of ether component (ppm)         | 22                                                     | 320                                                    | 25                                                     | 350                                                    | 3300                                                   |
|                               | Residual amount of styrene (ppm)                 | 15                                                     | 12                                                     | 20                                                     | 34                                                     | 42                                                     |
| Printing performance of toner | Shelf stability rate (%) at high temperature (%) | 0.5                                                    | 0.6                                                    | 1.1                                                    | 1.1                                                    | 21.5                                                   |
|                               | Continuous printing in NN environment (prints)   | 16,000                                                 | 15,000                                                 | 13,000                                                 | 12,000                                                 | 9,000                                                  |
|                               | Continuous printing in HH environment (prints)   | 15,000                                                 | 14,000                                                 | 12,000                                                 | 10,000                                                 | 7,000                                                  |
| Odor evaluation of toner      |                                                  | A                                                      | B                                                      | A                                                      | B                                                      | C                                                      |

The following can be found from the test results shown in Table 1. The toners of Comparative example 1 and Comparative example 2 were inferior in shelf stability at high temperature, could not stably hold the charge amount of toner and were inferior in printing durability under N/N and H/H environments since Comparative example 1 and Comparative example 2 did not use the quaternary ammonium base containing copolymer specified of present invention as the charge control resin.

Also, Comparative example 3 used the quaternary ammonium base containing copolymer specified of present invention as the charge control resin of the toner. However, since the residual amount of the ether component exceeded the range specified in the present invention, the toner of Comparative example 3 was inferior in shelf stability at high temperature and inferior in printing durability under the N/N and H/H environments.

27

2. The toner for developing electrostatic image according to claim 1, wherein the organic peroxide is a peroxy ester compound represented by the following Formula 1:

Formula 1:



wherein, each of R and R' is an alkyl group.

3. The toner for developing electrostatic image according to claim 2, wherein each of R and R' in the Formula 1 is an alkyl group having 6 or less carbons.

4. The toner for developing electrostatic image according to claim 3, wherein the peroxy ester compound represented by Formula 1 in which carbon number of R and R' is 6 or less is t-butylperoxy-2-ethylbutanoate represented by the following Formula 9, t-butylperoxy-pivalate represented by the following Formula 13 or t-hexylperoxy-pivalate represented by the following Formula 14:

Formula 9:



Formula 13:



Formula 14:



5. The toner for developing electrostatic image according to claim 1, wherein a molecular weight of the organic peroxide is 205 or less.

6. The toner for developing electrostatic image according to claim 1, wherein an added amount of the organic peroxide is in the range from 0.1 to 15 parts by weight with respect to 100 parts by weight of the monovinyl monomer.

7. The toner for developing electrostatic image according to claim 1, wherein the quaternary ammonium base containing copolymer is a copolymer comprising a repeating structural unit having quaternary ammonium base represented by the following Formula 2:

Formula 2:



wherein, R<sup>1</sup> is a hydrogen atom or a methyl group; R<sup>2</sup> is an alkylene group having 1 to 3 carbons;

28

each of R<sup>3</sup> to R<sup>5</sup> is independently an alkyl group having 1 to 6 carbons, a phenyl group or an aralkyl group having 1 to 12 carbons; X is a halogen atom, an alkyl sulfonate residue having 1 to 6 carbons, a benzenesulfonate residue or a paratoluene sulfonate residue.

8. The toner for developing electrostatic image according to claim 7, wherein a vinyl monomer unit and a (meth)acrylate monomer unit is contained as the repeating structural unit constituting the quaternary ammonium base containing copolymer besides the repeating structural unit having quaternary ammonium base represented by the Formula 2.

9. The toner for developing electrostatic image according to claim 1, wherein a containing amount of a repeating structural unit having quaternary ammonium base in the quaternary ammonium base containing copolymer is in the range from 0.05 to 12 wt %.

10. The toner for developing electrostatic image according to claim 1, wherein a copolymerization ratio (weight ratio) of a vinyl aromatic hydrocarbon monomer unit and a (meth)acrylate monomer unit contained as repeating structural units constituting the quaternary ammonium base containing copolymer is in the range from 70:30 to 90:10.

11. The toner for developing electrostatic image according to claim 1, wherein a weight average molecular weight "Mw" of the quaternary ammonium base containing copolymer is in the range from 2,000 to 50,000.

12. The toner for developing electrostatic image according to claim 1, wherein an added amount of the quaternary ammonium base containing copolymer is in the range from 0.01 to 20 parts by weight with respect to 100 parts by weight of a binder resin.

13. The toner for developing electrostatic image according to claim 1, wherein the toner is a core-shell type toner.

14. A method of producing a toner for developing electrostatic image comprising the steps of:

(1) a preparation process of a polymerizable monomer composition, in which a polymerizable monomer, a colorant, a quaternary ammonium base containing copolymer having a glass transition temperature "Tg" in the range from 70 to 100°C. as a charge control resin are mixed together to prepare a polymerizable monomer composition;

(2) a suspension process, in which after the polymerizable monomer composition is dispersed in an aqueous dispersion medium comprising a dispersion stabilizer, an organic peroxide as a polymerization initiator is added and droplets of the polymerizable monomer composition are formed so as to obtain a suspension;

(3) a polymerization process, in which a temperature of the suspension is raised for polymerization so as to obtain an aqueous dispersion liquid of a colored resin particle; and

(4) a stripping process, in which the aqueous dispersion liquid of the colored resin particle is subject to a stripping treatment,

wherein each residual amount of an ether component and styrene remaining in the toner for developing electrostatic image is respectively less than 500 ppm and less than 50 ppm.

15. The method of producing a toner for developing electrostatic image according to claim 14, wherein the organic peroxide is a peroxy ester compound represented by the following Formula 1:

Formula 1:



wherein, each of R and R' is an alkyl group.

**16.** The method of producing a toner for developing electrostatic image according to claim **15**, wherein each of R and R' in the Formula 1 is an alkyl group having 6 or less carbons.

**17.** The method of producing a toner for developing electrostatic image according to claim **14**, wherein a temperature of the stripping treatment in the (4) stripping process is a glass

transition temperature (Tg) of a binder resin comprising the colored resin particles or more and less than (Tg+75)° C.

**18.** The method of producing a toner for developing electrostatic image according to claim **14**, wherein time required for the stripping treatment is in the range from 0.5 to 40 hours.

**19.** The method of producing a toner for developing electrostatic image according to claim **14**, wherein a polymerizable monomer for forming a shell layer and a polymerization initiator for shell are added to the aqueous dispersion medium to which the colored resin particles to be a core particle are dispersed followed by polymerization.

\* \* \* \* \*